

## UNITED STATES PATENT OFFICE

2,491,649

## LUBRICANT COMPOSITION

Gordon W. Duncan, Westfield, and John C. Zimmer, Union, N. J., assignors to Standard Oil Development Company, a corporation of Delaware

No Drawing. Application February 9, 1946,  
Serial No. 646,706

14 Claims. (Cl. 252—33)

1

The present invention relates to the field of mineral oil lubricants generally, and more particularly to improved additives to be used in compounding engine oils, extreme pressure lubricants and cuttings oils.

Experience has shown that mineral lubricating oils, when used to lubricate modern internal combustion engines decompose, producing products which accumulate in various parts of the engine, such as on the rings and in the ring grooves in the form of a lacquer and/or carbonaceous deposits, which is probably responsible for ring sticking, causing loss of power and other indications of poor performance. The addition of certain types of metal derivatives of organic compounds is known to improve the properties of these oils, such as their oiliness characteristics and their detergent action in engines, particularly manifest in the maintenance of a clean engine condition during operation. Calcium and other polyvalent metal salts of petroleum or synthetic sulfonic acids are known to have oil detergent properties, but their use is limited due to their corrosive action on certain types of bearings. Mineral lubricating oils and emulsifiable oils are also used quite extensively for lubricating and cooling metal cutting tools. In metal cutting, the pressures which are developed between the cutting tool and the work and between the cutting tool and the metal chips exceed the film strength of mineral lubricating oil, and it has therefore been found necessary to incorporate in the mineral oil an agent having load-bearing characteristics commonly designated as an extreme pressure additive.

The principal object of the present invention is the provision of novel load-bearing compounds useful as extreme pressure additives in the compounding of cutting oils, emulsifiable oils, and E. P. lubricants. Another object is the conversion of polyvalent metal sulfonates of engine oil detergent characteristics into a non-corrosive form. These and other objects will be apparent to those skilled in the art upon reading the following description.

It has now been found that the metal salts of oil-soluble sulfonic acids generally, and particularly the metal salts of the preferentially oil-soluble petroleum oil sulfonic acids, may be given load-bearing characteristics and improved as engine oil detergents by reacting them with metal polysulfides. Particularly suitable sulfonate salts useful as starting materials for the purposes of the present invention are those of the alkali and alkaline earth metals, e. g. sodium, potassium,

2

calcium, magnesium, strontium and barium. However, other polyvalent metal sulfonates may be used, such as those of aluminum, iron, zinc, lead, cadmium, cobalt, nickel, etc. These sulfonate salts are available in the form of concentrates in oil containing from about 20 to about 70% of these particular sulfonate salts in oil. According to the present invention the metal sulfonate concentrate is reacted with a metal polysulfide to produce sulfonate salt compounds having excellent load-bearing properties, as well as improved engine bearing corrosion resistance. The reaction of the sulfonate with the polysulfide is carried out according to the procedure and 5 under the conditions described in copending application Serial No. 564,546, filed November 21, 1944, now Patent No. 2,467,176. Broadly, the method followed in carrying out the reaction is to mix the sulfonate concentrate with a polysulfide 10 in aqueous solution in the ratio, on a molal basis, of at least 1 mol of sulfonate salt per mol of metal polysulfide. The mixture is then heated to 250—325° F., preferably 300—310° F., to drive off the water and react the polysulfide 15 with the sulfonate salt after which the reaction product is filtered, if necessary, and cooled. In some cases it is desirable to include an alkaline reacting material to give an alkaline product. As an example, 0.1 mol of calcium hydroxide may 20 be included when treating calcium sulfonate with calcium polysulfide, or the reaction product may be reacted with calcium hydroxide. The type of metal polysulfide used in the reaction will depend to some extent upon the use to which the 25 final product is intended. If an E. P. additive and oil detergent is desired, it is preferred to use an alkaline earth metal polysulfide such as calcium, magnesium, strontium, or barium polysulfide, whereas if the product is to be used in 30 an emulsifiable cutting oil composition, an alkali metal polysulfide, such as sodium or potassium polysulfide, is reacted with the sulfonate salt concentrate.

It is believed that the polyvalent metal polysulfides when reacted with oil-soluble sulfonates give oil-soluble complex polyvalent metal sulfonates of the Werner type. For the production of a cutting oil, the oil-soluble concentrate of polyvalent metal sulfonate complex is blended 35 with a suitable lubricating oil base to yield a compounded oil containing 1 to 10% of the complex, e. g. when using a 30% concentrate, 3.3% of this material blended in the oil will furnish an oil containing 1% of the effective addition agents 40 and 33% will yield a blend containing 10% of

**E. P. additives.** Soluble oils are blended so as to contain from 2.0 to 20% of sulfonate polysulfide reaction products. As engine oil detergents the additives are blended with lubricating oil base stocks in concentrations between 0.02 and 5.0% and preferably from 0.1 to 2.5%. The exact amount of addition agent, within the limits prescribed, in each instance will depend upon the nature of the lubricating oil base stock, the general operating conditions and the result desired.

Having described the invention in its general aspects, the following examples will serve to illustrate specific applications thereof.

**Example 1**

200 grams of a solid 30% concentrate of preferably oil-soluble normal calcium sulfonate in oil, containing 1.25% calcium, 2.35% sulfur and 4.30% ash, was mixed with 10 grams of an aqueous solution of calcium polysulfide containing 6.82% calcium and 24.44% sulfur (an amount equivalent to 5% calcium polysulfide by weight of the calcium sulfonate in the original concentrate). After agitating to secure an intimate mixture, the temperature was raised to 300° F. to drive off the water. A clear, fluid, odorless product containing 1.54% calcium, 2.93% sulfur and 4.89% ash was obtained. 5% blends of this product and of the original untreated concentrate were made up in an extracted naphthenic lubricating oil and then tested for bearing corrosion life as follows: 500 cc. of the blend was placed in a glass oxidation tube (13" long and 2 $\frac{1}{2}$ " in diameter) fed at the bottom with a quarter inch bore air inlet tube perforated to facilitate air distribution. The oxidation tube was then immersed in a heated bath so that the oil temperature was maintained at 325° F. during the test. Two quarter sections of automotive bearings of copperlead alloy of known weight having a total area of 25 sq. cm. were attached to opposite sides of a stainless steel rod which was then immersed in the oil and rotated at 600 R. P. M., thus providing sufficient agitation of the sample during the test. Air was then blown through the oil at the rate of 2 cubic feet per hour for 4 hours. The bearings were then cleaned by washing with naphtha, dried and weighed and the loss in weight noted. The bearings were then repolished (to increase the severity of the test) reweighed and placed in the oil for another 4 hour period. The test in each case was continued in 4-hour periods until the accumulated loss in weight of the bearings exceeded 100 mg. The 5% blend of the original calcium sulfonate concentrate caused a bearing weight loss of 96 mg. after 4 hours and 285 mg. after 8 hours. The 5% blend of the reaction product caused no weight loss after 4 hours nor after 8 hours and only 31 mg. at 12 hours and 200 mg. after 16 hours.

**Example 2**

A blend was then made up in an extracted naphthenic lubricating oil containing 10% of the reaction product of Example 1 and tested on the Almen machine where it carried the full 15 weight load. A 10% blend of the original calcium sulfonate concentrate in the same extracted naphthenic lubricating oil failed at 3 weights in the Almen test. This test illustrates the unusual load-carrying properties of the calcium polysulfide product.

**Example 3**

As a further example of our invention, an emulsifiable oil of superior load-carrying ability can be prepared employing as the chief emulsifying agent a concentrate of preferably oil-soluble sodium sulfonate which has been reacted with sodium polysulfide. Such a concentrate was prepared as follows:

100 grams of a 50% oil solution of sodium sulfonate was emulsified with 35 grams of an aqueous solution of sodium polysulfide (1.9% preferably oil-soluble sodium, 6.5% sulfur) and heated to above 250° F. The resultant product was clear, odorless, and quite fluid.

15 Although the preferably oil-soluble metal sulfonates have been used to illustrate the principles of the present invention, metal phenates, phenol sulfides, metal derivatives of phenol sulfides and thiophosphates and their metal salts may also be greatly improved in their bearing corrosion characteristics by reacting them with metal polysulfides.

20 When the additives of the present invention are employed in crankcase lubricants their action may sometimes be enhanced by using them in conjunction with other additives such as metal soaps, metal phenates, metal alcoholates, metal phenol sulfides, organo substituted acids of phosphorus and metal salts of the same, metal xanthates, other sulfur or phosphorus compounds, nitrogen compounds, pour point depressors, V. I. improvers, oiliness agents and the like. Thus, the additives of the present invention may be used with one or more of the following representative materials:

25 Barium tert. octyl phenol sulfide  
Tin salt of wax alkylated phenol sulfide  
Calcium cetyl phenate  
30 Zinc isopropyl xanthate  
Aluminum naphthenate  
Barium di tert. amyl phenol sulfide  
Zinc tert. octyl phenol sulfide thiophosphate  
35 Magnesium lauryl salicylate  
Calcium phenyl stearate  
Zinc di-isopropyl salicylate  
40 Stearyl alcohol  
Tert. amyl phenol sulfide  
2,6-di tert. butyl-4-methyl phenol  
45 Polymerized lauryl methacrylate  
Sulfurized sperm oil  
Phenyl alpha naphthylamine  
Dibenzyl disulfide

50 In addition to their use in crankcase oils, extreme pressure lubricants and cutting oils, it is contemplated to employ the additives of the present invention in engine flushing oils, industrial oils, rust preventive compositions and greases.

55 What is claimed is:

1. A composition of matter consisting essentially of a major amount of a mineral lubricating oil and 0.02 to 10% by weight based on the total composition of the reaction product of at least one molecular proportion of a metal salt of preferentially oil-soluble petroleum oil sulfonic acid with one molar proportion of a metal polysulfide selected from the alkali and alkaline earth metal polysulfides, said reaction product being prepared 60 by mixing together a concentrate in mineral oil of said first named metal compound and an aqueous solution of said polysulfide and heating the mixture to a temperature ranging between 250° and 325° F. to complete said reaction and drive 65 off water.

2. A composition of matter consisting essentially of a major amount of a mineral lubricating oil and 0.02 to 10% by weight based on the total composition of at least one molecular proportion of a polyvalent metal of a preferentially oil-soluble petroleum oil sulfonic acid with one molecular proportion of a metal polysulfide selected from the alkali and alkaline earth metal polysulfides, said reaction product being prepared by mixing together a concentrate in mineral oil of said first named metal compound and an aqueous solution of said polysulfide and heating the mixture to a temperature ranging between 250° and 325° F. to complete said reaction and drive off water.

3. A composition of matter consisting essentially of a major amount of a mineral lubricating oil and 0.02 to 10% by weight based on the total composition of the reaction product of at least one molecular proportion of preferably oil-soluble calcium sulfonate with one molecular proportion of a metal polysulfide selected from the alkali and alkaline earth metal polysulfides, said reaction product being prepared by mixing together a concentrate in mineral oil of said first named metal compound and an aqueous solution of said polysulfide and heating the mixture to a temperature ranging between 250° and 325° F. to complete said reaction and drive off water.

4. A composition of matter consisting essentially of a major amount of a mineral lubricating oil and 0.02 to 10% by weight based on the total composition of the reaction product of at least one molecular proportion of the metal salt of a preferentially oil-soluble petroleum oil sulfonic acid with one molecular proportion of an alkaline earth metal polysulfide said reaction product being produced by mixing together a concentrate in mineral oil of said sulfonate and an aqueous solution of said polysulfide and heating the mixture to a temperature ranging between 250° and 325° F. to complete said reaction and drive off water.

5. A composition of matter consisting essentially of a major amount of a mineral lubricating oil and 0.02 to 10% by weight based on the total composition of the reaction product of at least one molecular proportion of a metal salt of preferentially oil-soluble petroleum oil sulfonic acid with one molecular proportion of calcium polysulfide said reaction product being produced by mixing together a concentrate in mineral oil of said sulfonate and an aqueous solution of said polysulfide and heating the mixture to a temperature ranging between 250° and 325° F. to complete said reaction and drive off water.

6. A composition of matter consisting essentially of a major amount of a mineral lubricating oil and 0.02 to 10% by weight based on the total composition of the reaction product of at least one molecular proportion of calcium sulfonate and preferentially oil-soluble calcium polysulfide said reaction product being produced by mixing together a concentrate in mineral oil of said sulfonate and an aqueous solution of said polysulfide and heating the mixture to a temperature ranging between 250° and 325° F. to complete said reaction and drive off water.

7. A cutting oil composition consisting essentially of a mineral lubricating oil and 1-10% of the reaction product of at least one molecular proportion of a polyvalent metal salt of a preferentially oil-soluble petroleum oil sulfonic acid with one molecular proportion of an alkaline earth metal polysulfide said reaction product being produced by mixing together a concentrate in mineral oil of said sulfonate and an aqueous

solution of said polysulfide and heating the mixture to a temperature ranging between 250° and 325° F. to complete said reaction and drive off water.

5. 8. A cutting oil composition consisting essentially of a mineral lubricating oil and 1-10% of the reaction product of at least one molecular proportion of preferentially oil-soluble calcium sulfonate with one molecular proportion of a calcium polysulfide said reaction product being produced by mixing together a concentrate in mineral oil of said sulfonate and an aqueous solution of said polysulfide and heating the mixture to a temperature ranging between 250° and 325° F. to complete said reaction and drive off water.

9. A cutting oil composition consisting essentially of a mineral lubricating oil and 3.5% of the reaction product of at least one molecular proportion of preferentially oil-soluble calcium sulfonate with one molecular proportion of calcium polysulfide, said reaction product being produced by mixing together a concentrate in mineral oil of said sulfonate and an aqueous solution of said polysulfide and heating the mixture to a temperature ranging between 250° and 325° F. to complete said reaction and drive off water.

10. An emulsifiable oil concentrate consisting essentially of a major proportion of a mineral lubricating oil and 1 to 10% by weight based on the total composition of the reaction product of at least one molecular proportion of sodium sulfonate with one molecular proportion of preferentially oil-soluble sodium polysulfide, said reaction product being produced by mixing together a concentrate in mineral oil of said sulfonate and an aqueous solution of said polysulfide and heating the mixture to a temperature ranging between 250° and 325° F. to complete said reaction and drive off water.

11. As a composition of matter the reaction product of at least one molecular proportion of a preferentially oil-soluble metal salt of a petroleum sulfonic acid with one molecular proportion of a metal polysulfide selected from the alkali and alkaline earth metal polysulfides, said reaction product being prepared by mixing together a concentrate in mineral oil of said first named metal compound and an aqueous solution of said polysulfide and heating the mixture to a temperature ranging between 250° and 325° F. to complete said reaction and drive off water.

12. As a composition of matter the reaction product of at least one molecular proportion of a preferentially oil-soluble polyvalent metal petroleum sulfonate with one molecular proportion of a metal polysulfide selected from the alkali and alkaline earth metal polysulfides, said reaction product being prepared by mixing together a concentrate in mineral oil of said first named metal compound and an aqueous solution of said polysulfide and heating the mixture to a temperature ranging between 250° and 325° F. to complete said reaction and drive off water.

13. As a composition of matter the reaction product of preferentially oil-soluble calcium petroleum sulfonate with one molecular proportion of a metal polysulfide selected from the alkali and alkaline earth metal polysulfides, said reaction product being prepared by mixing together a concentrate in mineral oil of said first named metal compound and an aqueous solution of said polysulfide and heating the mixture to a temperature ranging between 250° and 325° F. to complete said reaction and drive off water.

14. As a composition of matter the reaction product of preferentially oil-soluble calcium pe-

trolein sulfonate with one molecular proportion of calcium polysulfide selected from the alkali and alkaline earth metal polysulfides, said reaction product being prepared by mixing together a concentrate in mineral oil of said first named metal compound and an aqueous solution of said polysulfide and heating the mixture to a temperature ranging between 250° and 325° F. to complete said reaction and drive off water.

GORDON W. DUNCAN.  
JOHN C. ZIMMER.

## REFERENCES CITED

The following references are of record in the file of this patent:

## 5 UNITED STATES PATENTS

|    | Number    | Name         | Date          |
|----|-----------|--------------|---------------|
|    | 2,202,394 | Morway       | May 28, 1940  |
|    | 2,222,482 | Hagge et al. | Nov. 19, 1940 |
| 10 | 2,349,785 | Faust        | May 23, 1944  |
|    | 2,418,894 | McNab et al. | Apr. 15, 1947 |